

## UNITED STATES PATENT OFFICE

2,328,307

## MANUFACTURE OF RAYON

Gilbert I. Thurmond, Asheville, and Edward Brenner, Hendersonville, N. C., assignors to American Enka Corporation, Enka, N. C., a corporation of Delaware

No Drawing. Application April 5, 1940,  
Serial No. 328,146

7 Claims. (Cl. 18—54)

The present invention relates to the manufacture of rayon and more particularly to the production of viscose rayon thread of relatively high tenacity in both wet and dry state. Furthermore, viscose threads produced in accordance with the present invention, have very low elongations and other favorable properties useful in the weaving and analogous arts.

Up to the present time, the normal process for spinning rayon thread has involved the use of a single acid coagulating bath. As distinguished from the said single bath, the trend in the industry is to utilize the so-called "two-bath" spinning system. Such a system includes a primary coagulating and partial regenerating bath, and a second bath in which further regeneration of the thread is effected while a high stretch is simultaneously applied thereto. In order to carry out a relatively high degree of stretch, it has been found essential to maintain the said second bath at a relatively high temperature, i. e., above 60° C. and preferably in the neighborhood of 80° C. It is the general theory that this stretching, while passing the thread through a second bath during regeneration, orients the micelles in the individual filaments and thereby increases the strength or tenacity of the finished thread.

In the two-bath system normally employed, the coagulating bath contains an appreciable amount of sulphuric acid, as it is well-known that sulphuric acid effects both coagulation and regeneration of the thread. However, in order to impart a high degree of stretching in the second bath, the regeneration of the thread must be retarded in the first bath, because the thread in the form of its xanthate has considerably higher elasticity and extensibility. In other words, the extent to which the thread can be stretched varies inversely with the degree of regeneration. In order to retard the regenerative action of the acid in the first bath, it is necessary to add thereto, metallic salts such as sodium sulphate, zinc sulphate and magnesium sulphate. Obviously, the freshly extruded filaments constituting the thread must be sufficiently coagulated in order to elongate the same in the form of fine filaments and consequently, prior to the present invention, a concentration of at least 5% sulphuric acid has been used in the first bath.

*Explanatory note.*—In the prior art including patents and literature, the terms "coagulating" and "regenerating" have been used interchangeably and therefore, the meaning has been confused and misconstrued. The coagulation of viscose is a more or less physical change in the con-

version of the viscose solutions into filaments wherein the thread is still in the form of cellulose xanthate which is chemically similar to viscose. The regeneration of the xanthate is the decomposition or conversion of cellulose xanthate into pure cellulose.

Usually, 7% to 10% sulphuric acid is maintained in the first bath, and these amounts require a higher concentration of salts, zinc sulphate being the most effective salt for retarding the regeneration of the xanthate. However, the use of zinc is objectionable for a number of reasons, one of which is that zinc can only retard the regeneration to a limited extent.

15 It is the object of the present invention to either eliminate the use of sulphuric acid in the primary coagulating bath, or to use sulphuric acid in concentrations sufficiently low to prevent substantial regeneration of the cellulose xanthate even without employing metallic salts in conjunction therewith.

The invention further contemplates the utilization of a primary bath containing sufficient ammonium sulphate to coagulate viscose thread.

20 As a further object, the invention contemplates correlating the rate of regeneration of the cellulose xanthate with a high total stretch conducted in stages so as to provide a thread having a maximum degree of strength and a minimum elongation.

25 It has been determined in accordance with the present invention, that very low concentrations of sulphuric acid can be successfully used in the primary coagulating bath, so that it is not necessary to employ any zinc salts. As a matter of fact, we have unexpectedly found that if appreciable concentrations of ammonium sulphate be substituted in the first bath for sulphuric acid, then the use of metallic sulphates can be eliminated and the thread is sufficiently coagulated

30 without substantial regeneration, due to the absence of sulphuric acid. Sulphuric acid in very low concentrations, for example of from 1% to 3%, may even be used in conjunction with the ammonium sulphate for the purpose of neutralizing the alkalinity that would otherwise occur as a result of the alkaline thread being continuously introduced into the coagulating bath.

35 From the above it can be seen that satisfactory spinning of viscous filaments is possible with the omission of sulphuric acid or with sulphuric acid in very low concentrations in order to maintain a slight acidity in the bath and salts, if desirable, to retard the reaction rate of sulphuric acid with viscose. None of these salts contributes

to the spinning except in the negative capacity of the degree to which they inhibit the reaction of sulphuric acid. On the other hand, ammonium sulphate is capable of coagulating viscose without the aid of acid or other ingredients. (Other ammonium salts may possess the same properties.)

Theoretically, pure cellulose xanthate can be stretched to an almost unlimited extent, and as the regeneration proceeds, the ability to stretch is correspondingly decreased. Therefore, the use of ammonium sulphate as a coagulant, has certain advantages over sulphuric acid, because as pointed out above, sulphuric acid in any concentration will tend to regenerate cellulose xanthate. It is to be pointed out, however, that as regeneration proceeds, the thread becomes less plastic and therefore its ability to stretch decreases, but as the plasticity is lowered, the micelles in the filaments tend to be more effectively oriented by stretching. Therefore, in order to effect a maximum strength or tenacity without impairing any of the other characteristics of the thread, a definite relation and adjustment between the rate and degree of regeneration and stretch must be set up.

Consistent with the above principle, the present process provides for optimum spinning conditions. Using ammonium sulphate permits unlimited control and adjustment between the rate of regeneration and stretching, because it not only coagulates viscose similar to sulphuric acid, but retards regeneration similar to metallic salts and to that extent acts as a substitute for both. Now in order to set up the optimum spinning conditions, the freshly coagulated cellulose xanthate thread is stretched between several points during regeneration and while the thread is passed through one or more hot regenerating baths. A number of regenerating baths may be more suitable than one regenerating bath when used in conjunction with a primary bath that serves to coagulate and initiate the regeneration of the thread. It is generally conceded that at least one regenerating bath should be maintained at a high temperature because the temperature accelerates the rate of regeneration, and also effects some swelling of the thread whereby it can be more suitably stretched. In case one regenerating bath is used, its composition may be generally the same as that used in the normal two-bath system (sulphuric acid in the first bath), i. e., approximately 1% sulphuric acid plus salts brought over from the first bath. In the case of using several regenerating baths, the first regenerating bath may contain approximately 1% sulphuric acid and the succeeding baths contain increasing concentrations of sulphuric acid.

More particularly with respect to the first bath, ammonium sulphate is the fundamental ingredient. This salt is used to coagulate the viscose thread and may be used alone, provided it is present in sufficient quantities, for example, more than 20%. Continuous spinning is effected by adding only sufficient sulphuric acid to neutralize the alkali being brought in with the viscose. However, in order to represent the best conditions for the purposes of the present invention, from 1% to 3% sulphuric acid should be used, in which case, salts such as sodium sulphate and magnesium sulphate may also be employed. In any event, the ammonium sulphate content should not be less than from 8% to 10%. For example, in a bath containing 10% ammonium sulphate and 2% sulphuric acid, at least 20% sodium sul-

phate or equivalent salts should be used. Recapitulating, ammonium sulphate coagulates, the sulphuric acid maintains acidity and assists in coagulation, and sodium sulphate retards the regenerative action of the acid. It is obvious that by varying the relative concentrations of these ingredients, a thread of any desired degree of regeneration can be effected. The limits for practical use of these ingredients are:

|                   | Per cent |
|-------------------|----------|
| Ammonium sulphate | 8-30     |
| Sodium sulphate   | 8-20     |
| Sulphuric acid    | 0-10     |

Excellent baths are those in which the sum of the concentrations of the salts and acids is about 30%. In general, it is not possible to use 2% to 3% sulphuric acid without getting considerable regeneration, although it is possible if there is a very high total salt content. With most of the ammonium baths, a range of poor spinning occurs when from 3% to 6% sulphuric acid is employed. At concentrations higher than 6%, a well-regenerated thread is obtained which may be suitable for certain purposes, but in any case, the salt content must be preadjusted.

More particularly with respect to the second bath or succeeding baths, its or their purpose is to gradually regenerate or complete the conversion of the xanthate to pure cellulose while simultaneously stretching the thread. This is accomplished by sulphuric acid in the presence of salts if necessary. The bath may contain from 1% to 10% sulphuric acid, and the salt content will depend upon the rate of regeneration required. The salts may also control certain other characteristics of the finished thread such as strength, brittleness, and cross section of the individual filaments. Furthermore, the concentration of the second bath may be varied in accordance with the change in temperature. At higher temperatures, less acid is required. The bath should be above 60° C. and preferably, the bath is maintained in the neighborhood of 75° C. to 80° C. in order to assist the stretching operation. As previously stated, a higher temperature effects a swelling of the thread which permits a greater degree of stretching.

In order to effect a proper stretching when utilizing our ammonium bath system, it is obvious that a number of different types of systems may be employed. For example, the thread may be stretched at proper points by means of driven godets rotating at different peripheral speeds or by means of stepped rollers, or by means of freely rotatable rollers of different size. One system which has proved satisfactory is that disclosed in application Serial No. 324,727, filed March 18, 1940. In that system, the thread is stretched at a plurality of points in its path of travel between the spinneret and collecting device. More explicitly, a stepped godet located above the coagulating bath imparts the initial stretch and thereafter the thread is passed around a freely rotatable roller submerged in a hot regenerating bath and thence to a second stepped roller rotating at a higher peripheral speed than the first mentioned godet. It is obvious that the composition of the coagulating bath will determine the initial regeneration of the thread, the control of which is unlimited due to the use of ammonium sulphate. Between the godets a second stretch is imparted simultaneous with the passage of thread through the regenerating bath.

75 The stretching of the thread takes place during

its transition period from the xanthate form to the regenerated form whereby a certain adjustment of stretch takes place and provides a thread of maximum strength and minimum elongation.

All concentrations are calculated as parts by weight of the bath.

#### EXAMPLE

A viscose solution having a composition of 8% cellulose and 7% sodium hydroxide, was extruded through spinnerets to form a thread of 120 filaments and 275 denier. The thread was passed through a bath containing 14% ammonium sulphate, 20% sodium sulphate and 1.5% sulphuric acid. The bath was maintained at 45° C. After passing the thread through the bath, it was preliminarily stretched and then passed through a second hot bath containing 2% sulphuric acid and maintained at 75° C. while simultaneously imparting a second high stretch thereto. A number of threads were stretched in the foregoing manner, except that different degrees of stretch were imparted, and after collecting, after-treating, and drying, the following properties were ascertained:

Table

| Percent of stretch | Tenacity grams/100 denier |            |          |            |
|--------------------|---------------------------|------------|----------|------------|
|                    | Dry                       |            | Wet      |            |
|                    | Strength                  | Elongation | Strength | Elongation |
| 80.                | 330                       | 4.3        | 189      | 6.7        |
| 90.                | 332                       | 3.8        | 202      | 6.1        |
| 90.                | 336                       | 4.7        | 193      | 6.1        |
| 100.               | 336                       | 4.1        | 207      | 6.0        |
| 100.               | 332                       | 4.1        | 201      | 5.5        |
| 116.               | 351                       | 4.3        | 214      | 5.4        |

The present invention is not intended to cover the use of ammonium baths per se, as such baths have been known for a number of years. It is however, intended to cover the use of ammonium salt coagulating baths in combination with regenerating baths together with simultaneous stretching and a correlation of the rate of regeneration with stretching, so that a final thread is obtained having a dry tenacity substantially greater than 3 grams per denier and a dry elongation at the breaking point of less than 10%.

It is to be understood that viscose rayon is intended to cover staple fibers and also films and heavy denier yarns such as those used for reinforcing rubber-like articles, cords for fish lines, sails, tents and the like.

What is claimed is:

1. A process for the manufacture of viscose rayon having a dry tenacity greater than 3 grams/denier and an elongation at the breaking point of less than 10% which comprises spinning viscose filaments in a coagulating bath containing at least 10% ammonium sulphate, sulphuric acid in an amount less than 3% and sufficient metallic salts to retard the regenerative action of the sulphuric acid, and stretching the filaments during regeneration thereof in at least one hot bath containing only such sulphuric acid and salts as are carried over by the thread from the first bath, which bath is maintained at a temperature in a range of 75° C. to 80° C.

2. A process for the manufacture of viscose rayon having a dry tenacity greater than 3 grams/denier and an elongation at the breaking point of less than 10% which comprises spin-

ning viscose filaments in an aqueous bath consisting exclusively of more than 20% ammonium sulphate to effect coagulation without substantial regeneration of the filaments, and stretching the filaments during regeneration thereof in at least one bath containing from 1% to 10% sulphuric acid and metallic salts, which bath is maintained at a temperature above 60° C.

3. A process for the manufacture of viscose rayon having a dry tenacity greater than 3 grams/denier and an elongation at the breaking point of less than 10% which comprises spinning viscose filaments in a bath containing at least 8% ammonium sulfate, 1% to 3% sulphuric acid, and sufficient metallic sulphates to maintain a total bath concentration approximating 30%, to effect coagulation without substantial regeneration of the filaments, and stretching the filaments during regeneration thereof in at least one bath containing from 1% to 10% sulphuric acid and metallic salts, which bath is maintained at a temperature above 60° C.

4. A process for the manufacture of viscose rayon having a dry tenacity greater than 3 grams/denier and an elongation at the breaking point of less than 10% which comprises spinning viscose filaments in a bath containing approximately, 14% ammonium sulphate, 20% sodium sulphate and 1.5% sulphuric acid, to effect coagulation without substantial regeneration of the filaments while imparting a preliminary stretch thereto, passing the filaments to a second regenerating bath containing approximately 2% sulphuric acid and maintained at approximately 75° C. and simultaneously effecting a second high stretch during passage of the filaments through the said bath and finally collecting the filaments in package form.

5. A process for the manufacture of viscose rayon having a dry tenacity greater than 3 grams/denier and an elongation at the breaking point of less than 10% which comprises spinning viscose filaments in a bath containing approximately 14% ammonium sulfate, 20% sodium sulfate and 1.5% sulfuric acid, to effect coagulation without substantial regeneration of the filaments while imparting a preliminary stretch thereto, passing the filaments to a plurality of regenerating baths, the first of which contains approximately 1% sulfuric acid and the succeeding baths contain increasing concentrations of sulfuric acid and, therefore, are of successively greater regenerating power, and stretching the thread in each bath to an extent consistent with the degree of regeneration effected thereby until complete regeneration is effected.

6. A process for the manufacture of viscose rayon having a dry tenacity greater than 3 gram/denier and an elongation at the breaking point of less than 10% which comprises spinning viscose filaments in a bath containing only sufficient ammonium sulfate and sulfuric acid to effect coagulation without substantial regeneration of the filaments, said ammonium sulfate content being not less than 8%, passing the filaments to a plurality of regenerating baths, the first of which contains approximately 1% sulfuric acid and the succeeding baths contain increasing concentrations of sulfuric acid whereby the thread is regenerated to successively greater degrees, and stretching the thread in each bath to an extent consistent with the de-

gree of regeneration effected thereby until complete regeneration is effected.

7. A process for the manufacture of viscose rayon having a dry tenacity greater than 3 gram/denier and an elongation at the breaking point of less than 10% which comprises spinning viscose filaments in a bath containing only sufficient ammonium sulfate and sulfuric acid to effect coagulation without substantial regeneration of the filaments, said ammonium sulfate content being not less than 8%, passing the filaments to a plurality of regenerating baths, the first of which contains approximately 1% of sul-

furic acid and the succeeding baths contain increasing concentrations of sulfuric acid and, therefore, greater regenerating power, and stretching the thread in each bath, the amount of stretch applied in each bath diminishing as the thread is regenerated, the said amount of stretch applied in each bath being consistent with the degree of regeneration effected in said bath, the regeneration proceeding substantially to completion in the last bath.

GILBERT I. THURMOND.  
EDWARD BRENNER.